

[54] PHOTOFFLASH LAMP

[76] Inventor: Thomas B. McDonough, c/o Sylvania Electric Products Inc., Mon-toursville, Pa. 17754

[22] Filed: Nov. 20, 1970

[21] Appl. No.: 91,252

[52] U.S. Cl.....431/93

[51] Int. Cl.....F21k 5/02

[58] Field of Search .....431/93, 95; 149/31,  
149/32

[56] References Cited

UNITED STATES PATENTS

3,667,992 6/1972 Brown et al. ....431/93  
3,674,411 7/1972 Schaffer .....431/93  
2,291,983 8/1942 Pipkin .....431/95

2,791,111 5/1957 Gleim.....431/95  
3,521,983 7/1970 Fink et al. ....431/93  
3,521,984 7/1970 Fink et al. ....431/93

Primary Examiner—Carroll B. Dority, Jr.

Attorney—Norman J. O'Malley, Edward J. Coleman  
and Joseph C. Ryan

[57] ABSTRACT

A percussive-type photoflash lamp having a primer of the type comprising a wire anvil partially coated with fulminating material and coaxially supported within a tube in a manner providing a clearance between the coating of fulminating material and the inner wall of the tube. The fulminating material contains sodium chlorate as the oxidizer and is prepared by mixing an aqueous slurry containing red phosphorus with an aqueous solution of dissolved sodium chlorate.

4 Claims, 1 Drawing Figure



PATENTED MAY 22 1973

3,734,679



THOMAS B. McDONOUGH  
INVENTOR

BY *Edward Coleman*

AGENT

## PHOTOFASH LAMP

This invention relates to the manufacture of percussive-type photoflash lamps and more particularly to the composition of the charge of fulminating material employed therewith.

Generally speaking, a percussive-type photoflash lamp comprises an hermetically sealed, light-transmittin envelope containing a source of actinic light and having a primer secured thereto. More particularly, the percussive-type photoflash lamp comprises a length of glass tubing constricted to a tip at one end thereof and having a primer sealed therein at the other end thereof. The length of glass tubing which defines the lamp envelope contains a combustible, such as shredded zirconium foil, and a combustion supporting gas, such as oxygen. The primer comprises a metal tube and a charge of fulminating material on a wire anvil coaxially supported therein. Operation of the lamp is initiated by an impact onto the tube of the primer to cause deflagration of the fulminating material on the wire anvil up through the tube to ignite the combustible disposed in the lamp envelope.

Previous impact-sensitive fulminating materials for percussive flashlamps employed potassium chlorate as the oxidizer. The amount of potassium chlorate required in workable formulations exceeded the solubility of the oxidizer in the quantity of water used. The resultant saturated solution of oxidizer promoted crystal growth, both in the separately prepared oxidizer component as well as in finished pastes of fulminating material. The addition of sufficient water to dissolve all of the potassium chlorate would produce fluids with such low solids content that application of sufficient quantities of fulminating material, onto the primer anvil wire would be impractical on a production basis.

Crystal growth of the oxidizer is deleterious in this application as only several thousandths of an inch clearance exists between the anvil wire and the tube within which it is coaxially supported. The thickness of the fulminating material required for reliable deflagration is about 0.002 inch to 0.003 inch. A lump on the surface of the fulminating material protruding only a few thousandths of an inch may cause contact between the impact and abrasion-sensitive coating on the anvil wire and the wall of the surrounding tube. Mechanical shock or vibration causes deflagration of coating wherein such contact occurs.

An additional disadvantage in using potassium chlorate is that it must be milled to obtain a particle size of several microns diameter. Particles of a couple of thousandths inch diameter increase the coating thickness of the fulminating material and increase the danger of inadvertant ignition from tube-to-coating contact.

The usual technique employed in the preparation of impact-sensitive fulminating material is to blend all components except the oxidizer. A separate paste of oxidizer is prepared and mixed with the other components to produce the finished fulminating material just before use. The paste of potassium chlorate oxidizer suffers crystal growth after three to four weeks storage. This crystal growth is a cause for rejection of the batch, and the material is wasted.

One additional disadvantage to the use of potassium chlorate is that the mixed fulminating material paste will run only about two hours on the production equipment before crystal growth beings to take place. This makes it necessary to remove and discard the fluid left

at two-hour intervals. In addition, the dispensing devices must be thoroughly cleansed before refilling with fresh fulminating material paste. Up to fifty percent of the paste produced is discarded because of this crystalization.

In view of the foregoing, the principal object of this invention is to provide a paste of fulminating material, for the primer of a percussive-type photoflash lamp, which remains free of crystal growth during storage and use. Another object is to provide a more reliable percussive-type photoflash lamp. Another object is to provide an oxidizer component which may be prepared by dissolving a chlorate salt in water and which does not suffer crystal formation either before or after admixture with the other components of the fulminating material. A further object of the invention is to provide an improved method of preparing fulminating material in which a chlorate salt is dissolved in water to provide the oxidizer component, rather than by grinding or milling in aqueous media.

I have found that these objects can be achieved by the use of sodium chlorate as the oxidizer instead of potassium chlorate. In accordance with the invention, sodium chlorate, which is over seven times as water soluble as potassium chlorate, is completely dissolved in both the oxidizer component and the finished paste. Because sodium chlorate forms non-saturated solutions in workable formulations of oxidizer component and finished fluid, it will not crystallize and thereby permits longterm storage. Finished fluids of fulminating material using sodium chlorate can be used up to 16 hours on production equipment without crystal formation, as compared to the 2 hour limit of potassium chlorate oxidized compositions. This fact results in significant cost savings, as almost all of the fulminating material produced may be utilized without the need for rejection caused by crystal growth.

Potassium chlorate is usually preferred for use in fulminating materials as it is non-hygroscopic. Sodium chlorate is hygroscopic and, as such, loses sensitivity in formulations of fulminating material which are exposed to air. In addition, the water absorbed may cause decomposition of the other materials comprising the fulminating material. However, sodium chlorate can be used to advantage in the fulminating material for percussive flashlamps as the hermetically sealed structure of such lamps provides a dry atmosphere.

By way of specific example, the paste composition of an impact sensitive fulminating material according to the invention may comprise: 49.66 percent water, 28.46 percent titanium, 10.36 percent red phosphorus, 8.55 percent sodium chlorate, 1.85 percent hydroxyethyl cellulose, 0.73 percent sodium lignin sulfonate, 0.28 percent magnesium oxide, 0.05 percent sodium 2-ethylhexyl sulfate, 0.03 percent sulfur, and 0.03 percent trichlorophenol.

The paste, when dried, constitutes the impact-sensitive fulminating material. Of course, the invention is not limited to the quantities indicated, and additions, deletions or variations in composition may be made to suit given applications and sensitivity requirements. For example, the burning behavior of the dried residue varies greatly with the concentration of sodium chlorate used. Below about 5 percent sodium chlorate in the paste, impact sensitivity falls off rapidly, whereas a composition with over 50 percent sodium chlorate re-

sults in a charge which burns violently and yields a decreased light output from the flashlamp.

Other chlorate salts which have cations not catalytically reactive toward red phosphorus and which are soluble to the extent of 15 percent or greater by weight in water may be used; for example, calcium chlorate, lithium chlorate, magnesium chlorate, aluminum chlorate, and zinc chlorate. However, the extreme deliquescence of these materials may render their use in flashlamps more difficult with regard to drying and maintaining the coating dry prior to hermetic closure of the flashlamp. Similarly, phosphorus sesquisulfide may be used in place of red phosphorus, if desired, although a slight loss in sensitivity may be noted. Also, zirconium or boron may be substituted for titanium.

The method of preparing the above described fulminating material paste according to the invention comprises: (1) blending all of the denoted materials, except the chlorate, with some of the water to provide an aqueous slurry containing the phosphorus and titanium, etc.; (2) dissolving the chlorate in water to provide an aqueous solution thereof; and (3) mixing the phosphorus slurry and chlorate solution together. The aqueous slurry or red phosphorus, etc., and the oxidizer solution are stored separately and, in the interest of safety, are blended together just before use. Either of the components is relatively safe, even when dry; but when combined and dried, the resultant material burns on impact or abrasion.

In the accompanying drawing, the single figure is a 30 sectional elevational view of a percussive-type photoflash lamp with which a charge of fulminating prepared in accordance with this invention may be employed. The lamp comprises a length of glass tubing defining an hermetically sealed lamp envelope 2 constricted at one 35 end to define an exhaust tip 4 and shaped to define a seal 6 about a primer 8 at the other end thereof. The primer 8 comprises a metal tube 10 and a wire anvil 12 coated with a charge of fulminating material 14. A combustible such as filamentary zirconium 16 and a combustion-supporting gas such as oxygen are disposed within the lamp envelope. The wire anvil 12 is centered within the tube 10 and held in place by a crimp 18 just above the head 20 of the anvil. Additional means, such as lobes 22 on wire anvil 12, are also used to aid in stabilizing and supporting it substantially coaxial within the primer tube 10 and ensuring clearance between the

fulminating material 14 and the inside wall of the tube 10. A refractory bead 24, fused to the wire anvil 12 just above the inner mouth of the primer tube 10, eliminates burn-throughs and functions as a deflector to deflect and control the ejection of hot particles of fulminating material from the primer tube.

In conclusion, the present invention provides an oxidizer component which remains free from crystal growth both as prepared and in the finished fulminating material paste. The oxidizer component is readily prepared by dissolution of the chlorate salt in water. The resultant coatings of fulminating material 14 on anvil 12 are uniform, smooth and lump-free even after the paste has run on production equipment for sixteen 15 hours. Such smooth coatings help maintain sufficient clearance between the fulminating material 14 and the tube 10 wall so that inadvertent lamp ignitions from scuffed primer are prevented. The coating uniformity ensures high reliability of deflagration upon impact and minimizes inadvertent lamp ignition.

What I claim is:

1. A photoflash lamp comprising: an hermetically sealed, light-transmitting envelope; a quantity of filamentary combustible material located within said envelope; a combustion-supporting gas in said envelope; and a primer secured to and extending from one end of said envelope and in communication therewith, said primer including a tube sealed in said end of said envelope and having an exposed segment outside said envelope, a wire anvil located substantially coaxial within said tube, and a body of fulminating material located on said wire anvil intermediate its ends and on that segment of said wire anvil located in said exposed segment of said tube but spaced from the inside wall thereof, said fulminating material containing sodium chlorate.
2. The combination of claim 1 in which said fulminating material also contains red phosphorus.
3. The combination of claim 1 in which said fulminating material contains red phosphorus, titanium and sodium chlorate.
4. The combination of claim 3 in which said fulminating material further contains hydroxyethyl cellulose, sodium lignin sulfonate, magnesium oxide, sodium 2-ethylhexyl sulfate, sulfur, and trichlorphenol.

\* \* \* \* \*